

# United States Patent

[11] 3,615,512

[72] Inventors **Jacques Ducrocq;**  
**Daniel Gallois, both of Vincennes, France**  
[21] Appl. No. **768,155**  
[22] Filed **Oct. 16, 1968**  
[45] Patented **Oct. 26, 1971**  
[73] Assignee **Eastman Kodak Company**  
**Rochester, N.Y.**

2,230,977 2/1941 Ham..... 96/61  
2,857,275 10/1958 Land et al..... 96/61  
2,875,048 2/1959 Haist et al..... 96/61  
3,161,514 12/1964 Henn..... 96/95  
3,169,992 2/1965 Henn..... 96/61  
3,245,793 4/1966 Smith ..... 96/61

## OTHER REFERENCES

"Organic Silver-Complexing Agents for Photographic Monobaths" by Haist et al., Photographic Science and Engineering; Vol. 5, No. 4, July-Aug. 1961 pp. 198 to 203.

Primary Examiner—William D. Martin  
Assistant Examiner—William R. Trenor  
Attorneys—W. H. J. Kline and Gerald E. Battist

[54] **PHOTOGRAPHIC COMPOSITIONS AND PROCESS  
FOR STABILIZING IMAGE RECORDS WITH SAID  
COMPOSITIONS**  
**16 Claims, No Drawings**

[52] U.S. Cl..... **96/61**,  
96/29, 96/95  
[51] Int. Cl..... **G03c 5/38**,  
G03c 5/30  
[50] Field of Search..... **96/61, 95,**  
**29**  
[56] **References Cited**  
UNITED STATES PATENTS  
2,375,740 3/1945 Dearing..... **96/61**

**ABSTRACT:** Photographic compositions comprising (1) a silver halide developing agent, (2) a water-soluble silver halide solvent and (3) a weak silver halide complexing agent. In one embodiment the above composition can be used to rapidly develop or stabilize image records in silver halide emulsions which contain addenda which lower the rate of dissolution of silver halide in a potassium thiocyanate solution.

PHOTOGRAPHIC COMPOSITIONS AND PROCESS FOR  
STABILIZING IMAGE RECORDS WITH SAID  
COMPOSITIONS

This invention relates to new processes for obtaining stable images in silver halide compositions. In one aspect this invention relates to new compositions which can be used to obtain stable images in silver halide compositions. In another aspect this invention relates to means for obtaining stable image records in direct-print emulsions. In still another aspect this invention relates to novel monobaths for stabilizing image records in photographic compositions.

It is known in the art to stabilize image records in silver halide compositions and in particular in direct-print silver halide compositions by treating said records with developing solutions. However, in internally sensitive silver halide compositions which have surface latent image specks in the background areas, conventional developing solutions do not discriminate satisfactorily between the latent internal image and the surface latent image. This is especially true when certain halogen acceptors, development modifiers, antifoggants and the like are present in the silver halide composition which lower the development rate of latent internal image in a silver halide composition.

Therefore, it is an object of this invention to provide new means for obtaining stable image records in photographic compositions.

It is another object of this invention to provide new compositions for stabilizing image records in silver halide compositions.

It is another object of this invention to provide new monobath systems.

It is still another object of this invention to provide means for stabilizing image records in internally sensitive silver halide compositions.

It is still another object to provide means for obtaining stable image records and high discrimination (D<sub>max</sub>-D<sub>min</sub>) in internally sensitive silver halide emulsions.

We have now found that these and other objects of the invention can be accomplished with a developer composition comprising a silver halide solvent and a weak silver complexing agent. It is believed that the silver complexing agent forms a silver ion complex. The weak silver complexing agents of this invention all have the inherent characteristic property of not being capable of reducing silver halide to metallic silver. In one embodiment the weak silver complexing agent is additionally characterized in that it contains the ethenic group



such as benzene, toluene, aniline, etc. In another embodiment the weak silver complexing agent is additionally characterized as being a halogenated hydrocarbon. The complexing agents are also substantially free of mercaptan groups (or tautomers thereof) which would provide other predominant characteristics. In still another embodiment we have found that polyhydric compounds such as lactose, maltose, glucose, and the like can be added to said stabilizing compositions to improve image discrimination when stabilizing a silver halide image record.

The silver halide compositions which can be stabilized or developed according to this invention are those which are internally sensitive to electromagnetic radiation, i.e., light, X-rays, electrons, etc. Suitable silver halides include internally sensitive silver bromide, silver bromoiodide, silver chlorobromide, silver chlorobromoiodide, and the like. The preferred emulsions are those wherein the silver halide is predominantly silver bromide. In a typical embodiment preferred emulsions according to this invention have higher internal sensitivity than surface sensitivity. Typical suitable emulsions are disclosed in Davey et al., U.S. Pat. No. 2,592,250 issued Apr. 8, 1952; U.S. Pat. No. 3,206,316; Porter et al., U.S. Pat. No. 3,206,313, *Glaskides, Photographic Chemistry*, Vol. 1, pp. 75

31-32, *Fountain Press*, London; McBride, U.S. Pat. No. 3,271,157 issued Sept. 6, 1966, McBride, U.S. Pat. No. 3,287,137 issued Nov. 22, 1966, and Hunt, *Photographic Science and Engineering*, Vol. 5, No. 2, Mar.—Apr., 1961, pp. 104-108.

The so-called "internal image" emulsions can be used in the invention, such having silver halide grains wherein a predominant amount of the sensitivity is internal to the grains. Such internal image emulsions are those which, when measured according to normal photographic techniques by coating a test portion of the emulsion on a transparent support, exposing to a light intensity scale having a fixed time between  $1 \times 10^{16}$  and 1 second, bleaching 5 minutes in a 0.3 percent potassium ferricyanide solution at 65° F. in Developer B below (an "internal-type" developer), have a sensitivity, measured at a density of 0.1 above fog, greater than the sensitivity of an identical test portion which has been exposed in the same way and developed for 6 minutes at 68° F. in developer A below (a "surface-type" developer).

DEVELOPER A

|    |                                |         |
|----|--------------------------------|---------|
| 25 | N-Methyl-p-aminophenol sulfate | 0.31 g. |
|    | Sodium sulfite, desiccated     | 39.6 g. |
|    | Hydroquinone                   | 6.0 g.  |
|    | Sodium carbonate, desiccated   | 18.7 g. |
|    | Potassium bromide              | 0.86 g. |
|    | Citric acid                    | 0.68 g. |
|    | Potassium metabisulfite        | 1.5 g.  |
|    | Water to make 1 liter          |         |

DEVELOPER B

|    |                                |         |
|----|--------------------------------|---------|
| 35 | N-Methyl-p-aminophenol sulfate | 2.0 g.  |
|    | Sodium sulfite, desiccated     | 90.0 g. |
|    | Hydroquinone                   | 8.0 g.  |
| 40 | Sodium carbonate, monohydrate  | 52.5 g. |
|    | Potassium bromide              | 5.0 g.  |
|    | Sodium thiosulfate 10.0 g.     |         |
|    | Water to make 1 liter          |         |

The stabilizing or developing baths of this invention provide unexpected increases in the stabilizing or development rate of silver halide compositions which contain addenda which lower the dissolution rate of silver halides in potassium thiocyanate. In one embodiment of this invention direct-print compositions containing a halogen acceptor which lowers the rate of dissolution of silver halide in potassium thiocyanate can be effectively and quickly stabilized to form permanent image records having high image discrimination. Typical direct-print emulsions which are preferably stabilized according to this invention contain halogen acceptors such as 1-n-butyl-1,2,5,6-tetrahydro-1,3,5-triazine-4-thiol, 2,2,4-trimethyl-6-mercaptopo-metadiazine, 5-methyl-2-mercaptopo-oxazoline, phenyl thiosemicarbazide and dithiomalonamide.

The photographic elements processed according to the present invention can contain only latent images or they can contain visible image records, such as in the instance of a photodeveloped direct-print element. A permanent visible substantially uniform image record having good image discrimination will be obtained regardless of whether film is entirely photodeveloped to a visible image record or contains no visible image record.

The stabilizing or developing bath can contain a wide variety of compounds which reduce silver halide to silver. Typical developers include N-methyl-p-aminophenol sulfate, hydroquinone, 1-phenyl-3-pyrazolidone, 1-phenyl-4methyl-4'-hydroxymethyl-3-pyrazolidone, ascorbic acids, and the like or mixtures of the same. In a preferred embodiment the developing agent comprises 1-phenyl-3-pyrazolidone/hydroquinone or 1-phenyl-3-pyrazolidone/ascorbic acid. The developing compositions also can contain agents such as an-

hydrous sodium sulfite, stabilizing agents such as, for example, sodium or potassium carbonate amines or amino and  $\text{SO}_2$  clathrates and other agents such as antifogging agents commonly used in developer compositions.

The stabilizers or developers of this invention contain a silver halide solvent or fixing agent such as for example, water-soluble thiocyanates. In one embodiment the thiocyanates are used in combination with organic thioethers. Suitable organic thioethers include those which when utilized in aqueous solutions (60°C.) at 0.02 molar concentrations, are capable of dissolving more than twice the amount (by weight) of silver chloride than that which can be dissolved by water at 60°C. Typical preferred organic thioethers which can be used according to this invention contain at least one moiety wherein oxygen and sulfur are separated by an ethylene radical (e.g.,  $-\text{O}-\text{CH}_2\text{CH}_2-\text{S}-$ ). Generally, the subject thioethers have one to three thioether atoms ( $-\text{S}-$ ), although thioether compounds having more than three thioether atoms can be used. Typical thioethers are disclosed in McBride, U.S. Pat. No. 3,271,157 issued Sept. 6, 1966. These organic thioethers play also the part of weak complexing agents such as defined hereinafter. Typical thiocyanates useful according to the invention include potassium thiocyanate, sodium thiocyanate, ammonium thiocyanate, and the like. Generally, the water-soluble thiocyanate is present in concentrations of about 25 grams to about 500 grams per liter and preferably from about 150 grams to about 450 grams per liter. Other suitable fixing agents can also be used within the scope of the invention; however, the thiocyanates are the preferred fixing agents.

The weak silver complexing agents are all characterized by the common property of not being capable of reducing silver halide to metallic silver. The weak complexing agents are generally incorporated in the stabilizing or developer compositions in concentrations of about 1 gram/liter to about 150 grams/liter and preferably from about 10 grams/liter to about 100 grams/liter. Preferably the weak silver complexing agents are those compounds which can be additionally characterized as hydrocarbons having an ethenic group



halogen groups or combinations of these groups in the compound. In a preferred embodiment the weak silver complexing agents contain at least one halogen group and more preferably at least one halogen group and at least one ethenic group. In another embodiment the weak silver complexing agents contain at least two ethenic groups and more preferably at least three ethenic groups. Typical compounds useful in the invention which have the above characteristic properties are acyclic ethylene compounds such as trichloroethylene and the like; cyclic ethylene compounds such as dicyclopentadiene and the like; aromatic compounds such as benzene, toluene, m-aminophenol, aniline, anisol, benzoic acid, benzylamine, benzyl alcohol, benzyl aldehyde, chlorobenzene, bromobenzene, m-cresol, dimethyl benzylamine, xylenes, ethylbenzene, N-methyl aniline, m-phenylene diamine, resorcinol, salicylic aldehyde, o-toluidine, primary phenylethyl alcohol, 1-methyl-3-phenylpropylamine, phenylethylamine, and the like; unsaturated heterocyclic compounds such as lutiidines, 2- $\beta$ -phenylethyl isoquinolinium bromide and the like; halogenated compounds such as disclosed by L. J. Andrews and R. W. Keefer in J.A.C.S. Review 71, 3644-3647, 1949; 72, 3113-3116, 1950; 72, 5034-5037, 1950; 73, 5733-5736, 1951, which include halomethanes such as methyl iodide, diiodomethane, chloroform and the like; dihaloethylenes such as diiodoethylenes, dichloroethylenes and the like; halobenzenes such as chlorobenzene, diiodobenzenes and the like.

We have also found that polyhydroxy compounds can be effectively added to the above developing or stabilizing baths of this invention to increase the discrimination ( $D_{\text{max}}-D_{\text{min}}$ ) of the image record. In a preferred embodiment carbohydrates

are employed such as lactose, maltose, levulose, glucose, mannitol, dextrose and the like.

The essential ingredients of the stabilizing or developing composition according to this invention, namely the developers, the weak silver complexing agents and the silver halide solvent can be prepackaged in a kit in diluted, concentrated, or powder form and can be either mixed together or packaged individually for use in making the permanizing composition of this invention. Either one or all of the essential ingredients can also be coated in a separate layer on the photographic element which can subsequently be activated by an aqueous solution. The respective compositions are generally prepackaged individually and can be readily added to water to form a bath. Therefore, it is understood that kits prepared for making stabilizing or developing compositions comprising the essential ingredients of this invention are contemplated to be within the scope of this invention.

The stabilizing or developing baths of this invention are particularly useful to stabilize the image record in silver halide compositions containing addenda which lower the rate of dissolution of silver halides in potassium thiocyanate. For example, when a common silver halide emulsion is dipped into a 15/100 in mass of aqueous solution of potassium thiocyanate, at 20°C., for 1 minute, the proportion of dissolved silver halide is 94/100, as will be seen in the following example 1. By operating in the same manner, but with a silver halide emulsion, useful according to the invention, which contains 1-n-butyl-1,2,5,6-tetrahydro-1,3,5-triazine-4-thiol at a concentration of 3.63 moles per 100 moles of silver halide, one notes that only 70/100 of silver halides are dissolved.

However, this decrease in the speed of dissolution of the silver halides due to the addenda in the emulsion (i.e. for example, halogen acceptor in a direct-print emulsion), is inhibited by the presence of a weak silver complexing agent, such as previously defined, in the silver halide solvent solution. As will be seen in the following example 1, it suffices to add 15 ml. of a weak silver complexing agent such as benzylamine to 1 l. of a 15/100 potassium thiocyanate solution in order to pick up the 70/100 to 92/100 92/100 mass proportion of dissolved silver halides.

The invention can be further illustrated by the following examples of preferred embodiments thereof, although it will be understood that the examples are included merely for purposes of illustration and are not intended to limit the scope of the invention unless otherwise indicated.

#### EXAMPLE 1

Two photodevelopable photographic products are prepared such as samples No. 1 and No. 3 of example 6 of French Pat. No. 1,450,983. Sample No. 1 serves as a control (product I). Another product is also prepared from sample No. 1 to which, one adds 2-mercapto-imidazole to the amount of  $3.63 \times 10^{-2}$  mole per silver gram/atom (product II). Sample No. 3 (product III) contains 1-n-butyl-1,2,5,6-tetrahydro-1,3,5-triazinethiol in the emulsion of sample I with a concentration of  $3.7 \times 10^{-2}$  mole per mole of silver. A sample of the three preceding unexposed photographic products are dipped for 1 minute, respectively, into the following solutions I and another sample of the same products into the following solution II:

#### Solution I

|                                       |        |
|---------------------------------------|--------|
| Potassium Thiocyanate                 | 150 g. |
| Water (sufficient quantity to obtain) | 1 l.   |

#### Solution II

|                                       |        |
|---------------------------------------|--------|
| Potassium Thiocyanate                 | 150 g. |
| Benzylamine                           | 15 ml. |
| Water (sufficient quantity to obtain) | 1 l.   |

After this treatment, the quantities of silver remaining in the emulsion are measured after 1 minute of reaction at 20°C. The obtained results are the following.

TABLE I

|                                                                     | Product I<br>(Control) | Product<br>II | Product<br>III |
|---------------------------------------------------------------------|------------------------|---------------|----------------|
| Solution I<br>Undissolved silver<br>after treatment<br>(% in mass)  | 6                      | 6             | 30             |
| Solution II<br>Undissolved silver<br>after treatment<br>(% in mass) | 6                      | 12            | 8              |

The dissolution rate of silver halide in silver halide emulsion containing certain addenda (product III) is reduced in sodium thiocyanate solvent (solution I). This decrease in dissolving speed is practically inhibited by the addition of benzylamine to the potassium thiocyanate solution (solution II). Similar results are obtained when the emulsion contains 1-n-butyl-1,2,5,6-tetrahydro-1,3,5-triazine-4-thiol, 2,2,4-trimethyl-6-mercaptopetadiazine, 5-methyl-2-mercaptop-oxazoline, phenyl thiosemicarbazide, and dithiomalonamide.

In contradistinction, some addenda utilized in silver halide emulsions do not reduce the dissolution rate of silver halide when treated with a potassium-thiocyanate bath such as shown by product II.

#### EXAMPLE 2

Two series of three samples are prepared of photographic products such as those that are described in example 1.

The six samples are exposed through a 0.30 neutral density step tablet for  $10^{13}$  under a lighting of approximately 1000 1x, they are then photodeveloped for 5 minutes under a lighting of 540 lx, and finally, a first series of samples is treated in a control stabilizing developer such as developer F:

|                                                                |         |  |  |
|----------------------------------------------------------------|---------|--|--|
| Developer F (control)                                          |         |  |  |
| Water                                                          | 500 ml. |  |  |
| Celon E (tetrasodium salt of tetracetic ethylene-diamine acid) | 1 g.    |  |  |
| Anhydrous sodium sulfite                                       | 40 g.   |  |  |
| Methylenethioethanol $-SO_2$ (20% $SO_2$ )                     | 70 g.   |  |  |
| 1-phenyl-4-methyl-4-hydroxymethyl-3-pyrazolidone               | 2.2 g.  |  |  |
| Ascorbic acid                                                  | 12 g.   |  |  |
| Potassium thiocyanate                                          | 150 g.  |  |  |
| Water (Sufficient quantity to obtain)                          | 1 l.    |  |  |

The second series of samples is treated separately in a treatment monobath according to the invention (developer G) with the formula:

|                                                  |         |  |  |
|--------------------------------------------------|---------|--|--|
| Water                                            | 500 ml. |  |  |
| Celon E                                          | 1 g.    |  |  |
| Anhydrous sodium sulfite                         | 40 g.   |  |  |
| Methylenethioethanol $-SO_2$ (20% $SO_2$ )       | 70 g.   |  |  |
| 1-phenyl-4-methyl-4-hydroxymethyl-3-pyrazolidone | 2.2 g.  |  |  |
| Ascorbic acid                                    | 12 g.   |  |  |
| Potassium thiocyanate                            | 150 g.  |  |  |
| Benzylamine                                      | 15 ml.  |  |  |
| Water (sufficient quantity to obtain)            | 1 l.    |  |  |

The maximum density and the minimum density obtained with the product III according to the invention in developers F and G are the following:

TABLE II

| Monobath    | D <sub>max</sub> | D <sub>min</sub> | $\Delta D$ |
|-------------|------------------|------------------|------------|
| Developer F | 0.79             | 0.56             | 0.23       |
| Developer G | 0.69             | 0.25             | 0.44       |

It is noted that Product III treated in the new monobath embodied in the process according to the invention displays a more sizeable discrimination ( $\Delta D = D_{max} - D_{min}$ ) in spite of slight diminution of the  $D_{max}$ .

The following table III mentions, on the other hand, the quantities of developed silver and the covering power obtained with the six preceding samples.

TABLE III

| 15                                                   | Monobath | Product I        |                  | Product II       |                  | Product III      |                  |
|------------------------------------------------------|----------|------------------|------------------|------------------|------------------|------------------|------------------|
|                                                      |          | D <sub>min</sub> | D <sub>max</sub> | D <sub>min</sub> | D <sub>max</sub> | D <sub>min</sub> | D <sub>max</sub> |
| Developer F:                                         |          |                  |                  |                  |                  |                  |                  |
| Quantity of silver (mg./dm. <sup>2</sup> ) developed | 7.6      | 10.3             | 2.0              | 3.4              | 5.7              | 8.3              |                  |
| Covering power (log E/mg. silver)                    | 0.25     | 0.25             | 0.20             | 0.20             | 0.06             | 0.07             |                  |
| Developer G:                                         |          |                  |                  |                  |                  |                  |                  |
| Quantity of silver (mg./dm. <sup>2</sup> ) developed | 13.3     | 14.0             | 2.70             | 4.40             | 2.0              | 3.9              |                  |
| Covering power (log E/mg. silver)                    | 0.25     | 0.25             | 0.15             | 0.16             | 0.06             | 0.11             |                  |

Product I, treated in developer G (developer containing benzylamine) displays a quantity of developed silver clearly increased compared to that obtained in developer F.

Product II gives comparable results. The covering power, which remains high, is slightly diminished by the presence of benzylamine.

Product III displays results opposite to those obtained with products I and II. The treatment according to the invention provides a diminution of the quantity of developed silver. On the other hand, the quantity of silver developed in developer F (usual stabilizing developer) is clearly higher to that obtained with product II treated in the same bath. This result can be explained by the fact that 1-n-butyl-1,2,5,6-tetrahydro-1,3,5-triazine-4-thiol reduces considerably the fixing speed of the silver bromide through the potassium thiocyanate by forming a complex with the silver halide, as was seen in example 1. The role of the weak complexing silver agent such as the benzylamine of developer G is to inhibit this diminution of the dissolving speed of the silver halides in the potassium thiocyanate, as shown by example 1.

Similar results are obtained when utilizing 1-n-butyl-1,2,5,6-tetrahydro-1,3,5-triazine-4-thiol and 2,2,4-trimethyl-6-mercaptopetadiazine in Product III.

#### Example 3

This example shows that the association of an emulsion addenda, such as a halogen acceptor, and a weak complexing silver agent useful according to the invention makes it possible to inhibit the development of a surface image in a surface developer.

#### Developer H

|                                                             |          |
|-------------------------------------------------------------|----------|
| Formaldehyde bisulfite                                      | 61.2 g.  |
| Hydroquinone                                                | 14.45 g. |
| Boric acid                                                  | 5.5 g.   |
| Sodium sulfite                                              | 3 g.     |
| Quadratros (P <sub>2</sub> O <sub>5</sub> Na <sub>4</sub> ) | 1 g.     |
| Anhydrous sodium carbonate                                  | 71 g.    |
| Potassium bromide                                           | 2.8 g.   |
| Water (sufficient quantity to obtain)                       | 1 l.     |

A photographic product is prepared comprising a silver bromide photographic emulsion layer applied on a paper support, it is then exposed through a 0.15 neutral density step tablet for a microsecond by means of a flash bulb placed at 1 meter from the original (lighting of approximately 1 lumen per second). The photographic product exposed in this manner contains an internal image.

The photographic product is divided into five samples

which will be treated 5 minutes, respectively, in one of the following surface developers. These baths are prepared from developer H described above to which the compounds mentioned hereinafter are added. The results obtained are gathered in the following table IV.

TABLE IV

| Sample No. | Developer                                                                                                   | D <sub>max</sub> | D <sub>min</sub> | ΔD   |
|------------|-------------------------------------------------------------------------------------------------------------|------------------|------------------|------|
| 1          | (H) CONTROL                                                                                                 | 1.64             | 0.10             | 1.54 |
| 2          | (H)+0.2 g. of 1-phenyl-5-mercaptop-tetrazole per liter                                                      | 0.10             | 0.10             | 0    |
| 3          | (H)+0.03 g. of 2,2,4-trimethyl-6-mercaptopmetadiazine per liter                                             | 1.64             | 0.14             | 1.50 |
| 4          | (H)+N-methylaniline to the point of saturation                                                              | 1.60             | 0.16             | 1.44 |
| 5          | (H)+N-methylaniline to the point of saturation +0.03 g. of 2,2,4-trimethyl-6-mercaptopmetadiazine per liter | 0.10             | 0.10             | 0    |

With sample No. 2 which contains a usual antifogging agent which is also an inhibitor of nonselective development, a total inhibition of the development is noted. With sample No. 4, no inhibiting reaction of the development is noted due to N-methylaniline, weak complexing silver agent useful according to the invention. With sample No. 5, it is noted that the joint action of the compound of sample 3 and the N-methylaniline inhibits any development. Developer H being essentially a surface-image developer, the result obtained with sample No. 5 shows that the development of a surface image is inhibited.

Similar results are obtained by replacing in the preceding baths Nos. 3 and 5 the 2,2,4-trimethyl-6-mercaptopmetadiazine with 1-n-butyl-1,2,5,6-tetrahydro-1,3,5-triazine-4-thiol or other halogen acceptor useful according to the invention.

#### Example 4

This example shows that the association of certain addenda and a weak complexing silver agent useful according to the invention make it possible to develop an internal image in a solvent developer, without development of a surface image.

A photographic paper, such as that of example 3, is divided into five samples which are exposed as in example 4 and which are treated, respectively, in one of the developers mentioned in the following table V. These developers are prepared from developer I which develops at the same time both the internal and surface images; the other developers used for treating the various samples being derived from developer I to which the compounds mentioned in the following table V have been added.

#### Developer I

|                                |          |
|--------------------------------|----------|
| N-methyl-p-aminophenol sulfate | 1.85 g.  |
| Hydroquinone                   | 4.80 g.  |
| Boric acid                     | 0.83 g.  |
| Anhydrous sodium sulfite       | 18 g.    |
| Quadratofos                    | 2.40 g.  |
| Potassium bromide              | 0.74 g.  |
| 5-methyl-benzotriazole         | 0.032 g. |
| Anhydrous sodium carbonate     | 27.5 g.  |
| Anhydrous sodium thiosulfate   | 3.19 g.  |
| 2-benzoxazolethiol             | 0.025 g. |
| Water to make                  | 1 l.     |

TABLE V

| Sample No. | Developer  | D <sub>max</sub> | D <sub>min</sub> | ΔD   |
|------------|------------|------------------|------------------|------|
| 1          | I(control) | 1.60             | 0.12             | 1.48 |

|   |                                                                                                         |      |      |      |
|---|---------------------------------------------------------------------------------------------------------|------|------|------|
| 2 | I+0.2 g. of I-phenyl-5-mercaptop-tetrazole per liter                                                    | 0.12 | 0.12 | 0    |
| 3 | I+0.03 g. of 2,2,4-trimethyl-6-mercaptopmetadiazine per liter                                           | 1.48 | 0.14 | 1.34 |
| 4 | I+N-methylaniline to point of saturation                                                                | 1.55 | 0.18 | 1.37 |
| 5 | I+I+N-methylaniline to point of saturation +0.03 g. of 2,2,4-trimethyl-6-mercaptopmetadiazine per liter | 1.20 | 0.14 | 1.06 |

With sample No. 2, which contains a nonselective development inhibitor, a total inhibition of the development is noted, i.e., development inhibition of both the surface and internal image. With sample No. 3, an emulsion containing an addenda (halogen acceptor) used in small quantity makes it possible to obtain an image record very close to the control image record. With sample No. 5, no inhibition of the internal development is noted when the developer used contains a halogen acceptor and a weak silver complexing agent, useful according to the invention such as previously defined.

With this sample No. 5, a very legible image record is obtained which displays, compared with the control, only a slight diminution of the maximum density due to the surface development inhibition.

When N-methylaniline is replaced with other weak silver complexing agents, useful according to the invention and previously mentioned, a good inhibition of the surface image is noticed, while the internal image is well developed.

Similar results are obtained by replacing in the preceding baths nos. 3 and 5, the 2,2,4-trimethyl-6-mercaptopmetadiazine with 1-n-butyl-1,2,5,6-tetrahydro-1,3,5-triazine-4-thiol or any other halogen acceptor useful according to the invention.

The following example illustrates the application of the present invention to stabilizing treatment of photodevelopable copying papers which have been photodeveloped. Direct-print emulsions which have been exposed and photodeveloped, generally comprise two distinct images: an image essentially internal which displays the exposed part, i.e., image of interest, since it represents the sought information (it is also often called trace) and a background image due to the photodevelopment of the previously unexposed crystals. This background image is undesirable because an exposed and photodeveloped paper treated in a conventional internal developer develops the surface image or background image and reduces the discrimination ( $\Delta D = D_{max} - D_{min}$ ).

The present invention makes it possible to inhibit the development of the background image. Stabilizing developers according to the invention are used which develop the internal image without developing the background image. The use of this stabilizing developer also makes it possible to reduce treatment time necessary to stabilize a photographic element.

#### Example 5

A photodevelopable product is prepared by operating as in example 6 of French Pat. No. 1,450,953 (sample no. 3), but using 2,2,4-trimethyl-6-mercaptopmetadiazine as halogen acceptor in the amount of  $3.63 \times 10^{-2}$  mole per silver gram/atom, then by exposing through a 0.30 neutral density step tablet, for 1 microsecond by means of a flash bulb placed at 1 meter (lighting of approximately 1 lx. s). After photodeveloping for 5 minutes at 540 lx, this photographic product is divided in four samples which are treated for 1 minute respectively with one of the following treatment baths (developers J, C, D, E). Exposed but not photodeveloped samples are also treated with these developers.

Developer J has the following composition:

Developer J

|                                                                 |        |
|-----------------------------------------------------------------|--------|
| 1-phenyl-3-pyrazolidone                                         | 1.6 g. |
| Hydroquinone                                                    | 12 g.  |
| Anhydrous Sodium Sulfite                                        | 40 g.  |
| 2-methyl-aminoethanol, $\text{SO}_2$<br>(20% of $\text{SO}_2$ ) | 70 g.  |
| Potassium thiocyanate                                           | 150 g. |
| Potassium iodide                                                | 0.4 g. |
| Water (sufficient quantity to obtain)                           | 1 l.   |

Developer C

|                                                                 |        |
|-----------------------------------------------------------------|--------|
| 1-phenyl-3-pyrazolidone                                         | 1.6 g. |
| Hydroquinone                                                    | 12 g.  |
| Sodium sulfite anhydrous                                        | 40 g.  |
| 2-methyl-aminoethanol, $\text{SO}_2$<br>(20% of $\text{SO}_2$ ) | 70 g.  |
| Potassium thiocyanate                                           | 150 g. |
| Potassium iodide                                                | 0.4 g. |
| Benzylamine                                                     | 15 ml. |
| Water to make                                                   | 1 l.   |

Developer D

|                                                                |           |
|----------------------------------------------------------------|-----------|
| 1-phenyl-3-pyrazolidone                                        | 1.6 g.    |
| Hydroquinone                                                   | 12 g.     |
| Sodium Sulfite anhydrous                                       | 40 g.     |
| 2-methylaminoethanol, $\text{SO}_2$<br>(20% of $\text{SO}_2$ ) | 70 g.     |
| Potassium thiocyanate                                          | 150 g.    |
| Potassium iodide                                               | 0.4 g.    |
| Potassium bromide                                              | 4 a 16 g. |
| Benzylamine                                                    | 15 ml.    |
| Water to make                                                  | 1 l.      |

Developer E

|                                                                |          |
|----------------------------------------------------------------|----------|
| 1-phenyl-3-pyrazolidone                                        | 1.6 g.   |
| Hydroquinone                                                   | 12 g.    |
| Sodium Sulfite anhydrous                                       | 40 g.    |
| 2-methylaminoethanol, $\text{SO}_2$<br>(20% of $\text{SO}_2$ ) | 70 g.    |
| Potassium thiocyanate                                          | 150 g.   |
| Potassium iodide                                               | 0.4 g.   |
| Sodium thiosulfate                                             | 2 a 4 g. |
| Benzylamine                                                    | 15 ml.   |
| Water to make                                                  | 1 l.     |

Developer J is a usual developer for the internal image. If an exposed but not photodeveloped sample of the previously mentioned photographic product is developed chemically by such a developer, a copy is obtained with low Dmin and relatively high Dmax.

When the sample is photodeveloped, the Dmin increases due to the development of the surface image formed during the photodevelopment.

The stabilizing developers C, D, E according to the invention, when used on a photodeveloped sample, provide an image record identical to that obtained with a nonphotodeveloped sample (low Dmin and relatively high Dmax). The development of the surface image is apparently suppressed by the stabilizing developers.

Photodeveloped samples can be stabilized in developer J when benzylamine is added to obtain permanent images having density levels similar to those obtained with nonphotodeveloped samples treated by developer J above (usual internal developer).

Similar results are obtained when methyl iodide, benzene, N-methyl aniline, trichloroethylene, aminophenol, resorcinol, phenyl ethyl amine and the like are utilized in developer J for treating photodeveloped and nonphotodeveloped image records. EXAMPLE 6

Two samples are prepared from a photographic product such as described in example 5, which are exposed for one one-thousandths seconds behind a 0.30 neutral density step tablet (the lighting used is approximately 1 lx.s), and which is photodeveloped for 5 minutes at 540 lux. One of the samples is treated for 1 minute in developer F (control developer) of example 2.

The following densities are thus obtained:

$$D_{\min}=0.56 \quad D_{\max}=0.79 \quad \Delta D=0.23$$

5 The second sample is then treated for 1 minute in a stabilizing developer according to the invention similar to developer G of example 2 in which the benzylamine has been replaced with benzene at the point of saturation.

The results obtained are as follows:

$$D_{\min}=0.30 \quad D_{\max}=0.64 \quad \Delta D=0.34$$

EXAMPLE 7

This example illustrates the use of a halogenated compound 15 as a weak complexing silver agent for preparing a monobath according to the invention.

A sample according to example 6 is treated with the developer of example 6 wherein the benzene in the stabilizing developer has been replaced with methyl iodide at the point of 20 saturation.

The results obtained are as follows:

$$D_{\min}=0.34 \quad D_{\max}=0.81 \quad \Delta D=0.47$$

25 The incorporation of methyl iodide in the treatment monobath according to the invention makes it possible to increase considerably the ( $D_{\max}-D_{\min}$ ) as well as the visual contrast by the diminution of the Dmin.

EXAMPLE 8

Photographic elements are prepared with emulsions made according to French Pat. 1,450,983 which contains  $3.7 \times 10^{-12}$  mole per mole of silver of 1-n-butyl-1,2,5,6-tetrahydro-1,3,5-triazinethiol.

35 Samples of the photographic elements are made by exposure for one one-thousandth of a second behind a 0.30 neutral density step wedge and then photodeveloped for 5 minutes at 540 lumens.

The samples are treated in the following monobaths.

Monobath A      Monobath B,  
(control)

|                                                           |         |         |
|-----------------------------------------------------------|---------|---------|
| 45 Water                                                  | 500 ml. | 500 ml. |
| Celon E                                                   | 1 g.    | 1 g.    |
| Sodium Sulfite                                            | 40 g.   | 40 g.   |
| Methylaminoethanol- $\text{SO}_2$ (20% of $\text{SO}_2$ ) | 70 g.   | 70 g.   |
| 1-phenyl-3-pyrazolidone                                   | 2.2 g.  | 2.2 g.  |
| Ascorbic acid                                             | 12 g.   | 12 g.   |
| Potassium thiocyanate                                     | 150 g.  | 150 g.  |
| 1,8-dihydroxy-3,6-dithia-octane                           | 10 g.   | —       |
| Water to make                                             | 1 l.    | 1 l.    |

55 The samples are treated for 1 minute in the respective monobaths with the following results:

|                         | D <sub>max</sub> | D <sub>min</sub> | $\Delta D$ |
|-------------------------|------------------|------------------|------------|
| 60 Monobath A           | 0.73             | 0.43             | 0.30       |
| Monobath B <sub>1</sub> | 0.79             | 0.56             | 0.23       |

EXAMPLE 9

65 Carbohydrates can be used in combination with the weak silver complexing agents in the stabilizing or developing baths of this invention to provide synergistic improvements in the photographic properties of the image record.

Photographic elements are prepared according to example 70 1, exposed for one one-thousandth of a second behind a 0.30 neutral density step wedge and then photodeveloped for 5 minutes at 540 lux. One of the photographic elements is treated for 1 minute in monobath B<sub>2</sub> having the following composition:

Monobath B<sub>2</sub>

|                                                        |         |
|--------------------------------------------------------|---------|
| Water                                                  | 500 ml. |
| Celon E                                                | 1 gr.   |
| Sodium Sulfite                                         | 40 gr.  |
| 2-methyl aminoethanol                                  |         |
| SO <sub>2</sub> (20% SO <sub>2</sub> ) 2-methyl 70 gr. |         |
| 1-phenyl-3-pyrazolidone                                | 2.2 gr. |
| Ascorbic Acid                                          | 12 gr.  |
| Potassium thiocyanate                                  | 150 gr. |
| Potassium iodide                                       | 0.4 gr. |
| Water to make                                          | 1 l.    |

A second photographic element, prepared and exposed as above, is treated for 1 minute in a monobath according to monobath B<sub>2</sub> with the addition of 100 grams of saccharose per liter.

A third photographic element, prepared and exposed as above, is treated for 1 minute in a monobath according to monobath B<sub>2</sub> with the addition of 15 ml. of benzylamine per liter.

A fourth photographic element, prepared and exposed as above, is treated for 1 minute in a monobath according to monobath B<sub>2</sub> with the addition of 100 grams of saccharose and 15 ml. of benzylamine per liter.

The following results are obtained on a densitometer:

|          | D <sub>min</sub> | D <sub>max</sub> | ΔD   |
|----------|------------------|------------------|------|
| Sample 1 | 0.56             | 0.79             | 0.23 |
| Sample 2 | 0.56             | 0.79             | 0.23 |
| Sample 3 | 0.27             | 0.58             | 0.31 |
| Sample 4 | 0.25             | 0.63             | 0.38 |

It is apparent that the combinations of the carbohydrate and the weak silver complexing agent in the monobath provide an increase in D<sub>max</sub>, and a decrease in D<sub>min</sub>.

Similar results are obtained when the benzylamine is replaced with methyl iodide, benzene, N-methyl aniline, trichloroethylene, aminophenol, resorcinol, phenyl ethyl amine and the like.

## EXAMPLE 10

A photographic element, prepared and exposed as in example 9, is treated for 1 minute in a monobath according to monobath B<sub>2</sub> additionally containing 15 ml. of benzylamine and 100 grams of lactose per liter. The following results are obtained:

|          | D <sub>max</sub> | D <sub>min</sub> | ΔD   | sensitivity |
|----------|------------------|------------------|------|-------------|
| Sample 5 | 0.24             | 0.66             | 0.42 | 3.06        |

Similar results are obtained when maltose, levulose, glucose, amidon, mannitol and dextrose are used in the monobath in combination with the weak silver complexing agent.

The invention has been described in considerable detail with reference to preferred embodiments thereof, but is not limited to these.

be understood that variations and modification can be effected within the spirit and scope of the invention as described hereinabove and as defined in the appended claims.

We claim:

5. 1. A photographic monobath composition for developing direct-print photographic compositions comprising (1) a silver halide developing agent, (2) a water soluble thiocyanate silver halide solvent and (3) a weak silver halide complexing agent which is not capable of reducing silver halide to metallic silver.

10. 2. A photographic bath according to claim 1 wherein said weak silver halide complexing agent comprises at least one



group or halogen group.

15. 3. A photographic bath according to claim 1 wherein said silver halide solvent is potassium thiocyanate.

4. A photographic bath according to claim 1 wherein said weak silver halide complexing agent is an aromatic compound.

25. 5. A photographic bath according to claim 1 wherein said weak silver halide complexing agent is a halogenated organic compound.

6. A photographic bath according to claim 1 wherein said weak silver halide complexing agent is an organic thioether.

30. 7. A photographic bath according to claim 6 wherein said organic thioether comprises at least one moiety of the formula  $-\text{O}-\text{CH}_{2\text{bq2}}-\text{CH}_2-\text{S}-$ .

8. A photographic bath according to claim 1 wherein said developing agent comprises 1-phenyl-3-pyrazolidone/hydroquinone.

35. 9. A photographic bath according to claim 1 wherein said developing agent comprises 1-phenyl-3-pyrazolidone/ascorbic acid.

10. A photographic bath according to claim 1 wherein said 40 weak silver complexing agent comprises at least two ethenic groups.

11. A photographic bath according to claim 1 wherein said weak silver complexing agent contains a halogen group.

12. A photographic bath according to claim 11 wherein said 45 weak silver complexing agent further agent further contains an ethenic group.

13. A photographic bath according to claim 1 wherein said weak complexing agent comprises at least three ethenic groups.

50. 14. A photographic bath according to claim 1 further comprising a carbohydrate.

15. A photographic bath according to claim 1 wherein said weak silver complexing agent is benzylamine.

16. A photographic composition according to claim 1 55 wherein said weak silver complexing agent is substantially free of mercaptan groups.

\* \* \* \* \*

UNITED STATES PATENT OFFICE  
CERTIFICATE OF CORRECTION

Patent No. 3,615,512 Dated October 26, 1971

Inventor(s) Jacques Ducrocq and Daniel Gallois

It is certified that error appears in the above-identified patent and that said Letters Patent are hereby corrected as shown below:

Column 2, line 12, " $1 \times 10^{16}$ " should read  $---1 \times 10^{-6}---$ ; line 42, "10.0 g" should be directly under  $---5.0 g---$ ; line 56, "tetrachydro" should read  $---\text{tetrahydro}---$ . Column 3, line 1, "sulfite" should read  $---\text{sulfate}---$ . Column 4, line 51, after "1,450,983", please insert  $---$ ; lines 53 and 54, " $3.63 \times 10^{12}$ " should read  $---3.63 \times 10^{-2}---$ ; line 57, " $3.7 \times 10^{12}$ " should read  $---3.7 \times 10^{-2}---$ . Column 5, line 18, "(produce III)" should read  $---(\text{Product III})---$ ; line 36, " $10^{13}$ " should read  $---10^{-3}---$ ; line 43, "40 40" should read  $---40 \text{ g.}---$ . Column 8, line 67, " $3.63 \times 10^{12}$ " should read  $---3.63 \times 10^{-2}---$ . Column 10, lines 33 and 34, " $3.7 \times 10^{12}$ " should read  $---3.7 \times 10^{-2}---$ . Column 11, line 7, "70 gr." should be directly under  $---40 \text{ gr.}---$ . Claim 6 should be changed to read as follows:

Claim 7, line 3, " $(-\text{O}-\text{CH}_2-\text{bq}_2-\text{CH}_2-\text{S}-)$ " should read  $---(-\text{O}-\text{CH}_2-\text{CH}_2-\text{S}-)-$

Signed and sealed this 13th day of June 1972.

(SEAL)

Attest:

EDWARD M.FLETCHER, JR.  
Attesting Officer

ROBERT GOTTSCHALK  
Commissioner of Patents